

# United States Patent

[11] 3,627,737

[72] Inventor **Ralph W. Smith**  
Gulf Breeze, Fla.  
[21] Appl. No. **785,370**  
[22] Filed **Dec. 19, 1968**  
[45] Patented **Dec. 14, 1971**  
[73] Assignee **Monsanto Company**  
St. Louis, Mo.

Primary Examiner—Donald E. Czaja  
Assistant Examiner—V. P. Hoke  
Attorneys—Stanley M. Tarter and John W. Whisler

**ABSTRACT:** Aromatic polyamides are advantageously viscosity-stabilized by the presence during polymerization of a stabilizing amount of a compound of the formula:



wherein R is hydrogen, a lower alkyl radical or an aryl radical. The inherent viscosity of the polyamide is in the range of 0.8 and 2.4. Filaments wet-spun from such polyamide show improved tensile strength and resistance to abrasion.

[54] **FILAMENTS WET-SPUN FROM VISCOSITY-STABILIZED AROMATIC POLYAMIDES**  
3 Claims, No Drawings

[52] U.S. Cl. .... **260/78 R,**  
260/32.6 N, 260/45.9 R

[51] Int. Cl. .... **C08g 20/38**

[50] Field of Search. .... **260/45.9,**  
32.6 N, 78 R; 264/210 F

[56] **References Cited**

UNITED STATES PATENTS

3,049,518 8/1962 Stephens ..... **260/78**

## FILAMENTS WET-SPUN FROM VISCOSITY-STABILIZED AROMATIC POLYAMIDES

## BACKGROUND OF THE INVENTION

For more than three decades it has been known that high molecular weight polyamides capable of being formed into useful strands including films, fibers and the like can be prepared by heating certain amino acids or by heating certain diamines with dibasic carboxylic acids under polyamidation conditions. Aliphatic polyamides produced from polymers of 6aminocaproic acid and polymers of hexamethylene diamine and adipic acid have found wide spread acceptance in the textile industry. Commonly these polymers are referred to as nylon-6 and nylon-66, respectively.

These polyamides have melting points normally above 200° C. but below 280° C. For most textile purposes these melting points are quite acceptable. However, with the advent of use of fibers in the aerospace activities and other areas where extraordinary hot environment is present, filaments having much higher melting points were required. To meet this need wholly aromatic polyamide strands have been produced. While the aliphatic polyamides can be spun by the melt spinning process, the so-called wholly aromatic polyamides have such a high melting point that in order to produce filaments therefrom one must resort to using the wet spinning process with its attending disadvantages.

As is well known wet spinning involves dissolving the polymer in a suitable solvent and extruding the resulting solution in a coagulation bath wherein the polymer precipitates as filaments and the solvent is extracted from the extruded streams. It was found that by using solutions of aromatic polymer, solvent removal during wet spinning was encountered with much difficulty. It was noted that during coagulation a rather impervious skin developed on the forming filaments. This presence of skin hindered solvent removal from the inner core of the filaments. The filaments were low in tensile strength and abraded easily during use.

## SUMMARY OF THE INVENTION

An aromatic polyamide having been viscosity-stabilized with a small amount of a compound of the formula:



wherein R may be the same or different radicals selected from the group consisting of hydrogen, lower alkyl of one to six carbon atoms and aryl with an inherent viscosity of 0.8-2.4 can be produced. Filaments having fiber-forming properties made from these polymers by conventional wet spinning techniques exhibit improved strength and abrasion resistance.

## **DETAILED DESCRIPTION**

It has been found that aromatic polyamide strands of improved strength and abrasion resistance can be obtained by preparing such polyamides in the presence of a small amount of certain formamides whose chemical formulas have been structurally presented above, generally in the range of 0.204-1.63 percent based on the weight of the polymer. However, it has been found that fibrils useful in the manufacture of dielectric paper and composite materials can be formed more readily by including formamides in the range above 1.63 percent up to 4.0 percent by weight of the polymer. Tensile strength in the range of 5-8 grams per denier are obtainable when the end uses of the strands require strength. It is also possible that the strength be 1-5 grams per denier for end uses not requiring better tensile properties.

The polyamide useful in the practice of the invention is referred to herein as aromatic polyamides. This term refers to polymers wherein repeating units are linked together by a carbonyl group, i.e., the radical:



5 The amine and the carbonyl of each repeating carbonamide radical is directly attached to a carbon atom in the ring of an aromatic radical. The term aromatic radical means a carbocyclic ring possessing resonance. Thus included are all resonance-stabilized ring systems whether benzene-aromatic or hetero-aromatic. They may be single, multiple or fused ring structures. Exemplary aromatic radicals are



35 in which R is preferably a lower alkyl, lower alkoxy or halogen, n is a number from 0-4 inclusive, and X is preferably one of the groups



where Z is hydrogen or lower alkyl. X may also be lower alkylene or alkylene dioxy. R may also be nitro, lower carbalkoxy or other non reactive group. All of these aromatic radicals are divalent and are meta or para oriented.

Examples of preferred such polymers include those with the following recurring units:



poly-N,N'-m-phenylenebis(m-benzamide)4,4'-biphenyldicarbonamide



poly-4,4'-bis(p-aminophenyl)-2,2'-bithiazole isophthalamide



poly-2,5-bis(p-aminophenyl)-1,3,4-oxadiazole isophthalamide



poly-3,4'-diaminobenzanilide isophthalamide



and poly-4,4'-diaminobenzanilide terephthalamide



The process of preparing the polymer of the invention is conveniently conducted by known interfacial or solution polycondensation technique. The latter is preferred and involves dissolving a wholly aromatic diamine of the formula



where Y is selected from

a.  $-COHN-Ar-NHCO-Ar-$ 

and

b.  $-NHCO-Ar-COHN-Ar-$ 

where Ar is an aromatic radical of six through 16 carbon atoms and n is 0 to 1 inclusive, in a suitable solvent substantially inert to the polymerization reaction. Among such solvents are N,N-dimethylacetamide, 1-methyl-2-pyrrolidone, 1,5-dimethyl-2-pyrrolidone, hexamethylphosphoramide. These solvents are rendered more effective in many instances by mixing with them a small amount, up to 10 percent of an alkali or alkaline earth salt, such as lithium chloride, lithium bromide, magnesium chloride, magnesium bromide, beryllium chloride or calcium chloride. The preferred solvents for solution polymerization are N,N-dimethylacetamide or dimethylacetamide containing 5 percent lithium chloride. The temperature of the solution is lowered to between plus 10° and minus 20° C.; and an aromatic diacid halide of the formula:



wherein Ar is divalent aromatic radical and Hal is a halogen

atom selected from the group of chlorine, bromine and iodine, the first mentioned halogen being preferred, is added to the diamine solution along with a sufficient amount of proton acceptor and the mixture stirred continuously until the reaction is complete, the time depending upon the type of polymerization system and the polymer being prepared. Reaction is generally complete within a few minutes to a few hours.

Before the reaction is complete and preferably before the reaction is initiated the formamide viscosity stabilizer is added. Representative examples of specific formamide suitable for purpose of this invention are formamide; N-methyl-formamide; n,N-dimethylformamide (the most preferred); N-ethylformamide; N,N-diethylformamide; N-methyl-N-ethyl-formamide; N,N-di-n-propylformamide; N-ethyl-N-phenyl formamide; and others.

The amount of formamide stabilizer employed is critical and determines the ultimate spinning and fiber properties of the product. When the aromatic polyamide is to be employed for making filaments and the like quantities of formamide stabilizer should be at least 0.204 percent and normally not in excess of 1.63 percent by weight based on the weight of the polymer. The preferred range is 0.53 percent to 1.22 percent. Below 0.204 percent the viscosity of the polyamide is not appreciably affected with the result that the advantages of the present invention are not utilized to the fullest extent. Wet spun filaments made from aromatic polyamides viscosity-stabilized with less than 0.204 percent material have reduced abrasion resistance. If used in excess of 1.63 percent, the formamide stabilized aromatic polyamides are not suitable for fiber-forming material but may be used for film and coating material. When used in excess of 2.55 percent, the polymerization of the material has been so limited that the polymer has substantially no known utility except perhaps as a yarn sizing ingredient. The viscosity of the polymer is related to the amount of stabilizer added. Where dimethylformamide is employed in an amount of 0.204 to 1.63 percent, the inherent viscosity of the polymer is about 1.65-2.4. For amounts of 0.53-1.22 percent, the inherent viscosity is 1.8-2.2. And when 2.55 percent dimethylformamide is used, the aromatic polyamide has an inherent viscosity of only 1.4. Inherent viscosity is determined in accordance with the following equation.

$$\eta_{inh} \text{ (inherent viscosity)} = 1 \eta_{rel}/C$$

45 The relative viscosity ( $\eta_{rel}$ ) is determined by dividing the flow time in a capillary viscometer of a dilute solution of the polymer by the flow time for the pure solvent. The concentration (C) is generally 0.5 gram of polymer per 100 ml. of solution. The measurements are made at 22° C. in N,N-dimethylacetamide containing 5 percent lithium chloride.

## EXAMPLE I

55 Into a three liter polymerization vessel equipped with an efficient agitator, inert gas bleed device, and a drying tube were placed 209 grams of m-phenylene bis-(m-aminobenzamide) and 57 grams calcium carbonate. The vessel was flushed with nitrogen gas. To this mixture was added 1,300 ml. of high purity N,N-dimethylacetamide containing 0.03 percent dimethylformamide (0.122 percent based on the weight of the polymer). The resulting mixture was stirred until solution of the diamine was effected and was cooled to -20° C. by means of a dry ice and acetone bath. Agitation was again started and 122 grams of purified terephthaloyl chloride was added. As the viscosity and temperature gradually increased, the stirrer speed was decreased to provide proper mixing. The hydrogen chloride of reaction was neutralized with the added calcium carbonate by raising the reaction temperature to 80° C. The inherent viscosity of the polymer was determined to be 2.50.

70 The polymer containing solution was pumped with some difficulty through a multi-hole spinneret submerged in an aqueous spin bath. The resulting filaments were withdrawn from the bath and subjected to after treating steps of washing, draw-

ing, and drying. The average tenacity was 3.8 grams per denier at 30 percent break elongation. A sample fabric was made from the filaments and subjected to a standard abrasion test. It was found that the fabric was easily fibrillated. Upon microscopic analysis of the yarn a hard outer skin and soft core effect was observed. A method for showing the skin and core of a filament is generally described in Textile Research Journal, 1945, page 443.

#### EXAMPLE II

Example I was repeated with the exception that the dimethylacetamide solvent contained 0.30 percent N,N-dimethylformamide (1.22 percent based on polymer weight). The polymer had an inherent viscosity of 1.84. It was found that fabric made from the wet spun resulting filaments had improved strength of 5.8 g./d at 16 percent break elongation and improved abrasion resistance. Microscopic analysis of the yarn showed a less pronounced skin-core effect.

#### EXAMPLE III

Example I was repeated with the exception that N,N-dimethylformamide was added to increase the concentration to 0.60 percent. The polymer had an inherent viscosity of 1.44. It was found that fabric made from the resulting filaments had improved abrasion resistance. Microscopic analysis of the yarn showed a substantial absence of any skin-core effect.

#### EXAMPLE IV

Example I was repeated with the exception that the solvent contained 0.48 percent N,N-dimethylformamide. The resulting polymer had an inherent viscosity of 1.79. It was again found that fabric made from the resulting wet-spun filaments had excellent abrasion resistance.

#### EXAMPLE V

Example I was repeated with the exception that the solvent contained only 0.01 percent N,N-dimethylformamide (0.04 percent based on polymer weight). The resulting polymer had an inherent viscosity of 2.36. Difficulty was encountered in extruding the polymer solution to form fibers because of the occurrence of gelatinous polymeric particles. It was again found that fabric made therefrom had unsatisfactory resistance to abrasion.

#### EXAMPLE VI

Into the apparatus described in example I were placed 104.5 grams of m-phenylene bis(m-aminobenzamide) and 650 ml. of high purity N,N-dimethylacetamide. Calcium carbonate, 28.6 grams, was added and the mixture was cooled to -20° C. Just prior to the addition of 60.9 grams of the terephthaloyl chloride, 4.0 grams of formamide was added. The aromatic diacidchloride was then added and the polymerization was completed as described in example I. It was found that the presence of the dimethylacetamide effectively regulated the molecular weight of the polymer.

Likewise, when other aromatic polyamides are prepared in the presence of a suitable amount of other formamides within

the scope of the present invention, one produces polymers having reduced inherent viscosity. Filaments made therefrom have increased tensile properties and abrasion resistance.

As can be seen, an important aspect of the present invention is the regulation of the molecular weight of aromatic polyamides by the use of relatively low cost N,N-dialkyl formamides. Among the advantages of regulating the molecular weight of such polyamides are: to allow the use of high solids concentrations of polymer solutions which facilitate the spinning of high-strength fibers; to prevent uncontrolled polymerization resulting in the formation of undesirable gel formations; and to control the molecular weight of the polymer within a given range so that changes in spinning variables are not needed for producing a consistently high-quality fiber.

I claim:

1. A wet-spun filament having improved tensile properties and abrasion resistance made from an aromatic polyamide viscosity-stabilized with a compound of the formula:



wherein R is selected from the group consisting of hydrogen, lower alkyl of one to six carbon atoms, and aryl, the inherent viscosity of the polymer being in the range of 1.65 and 2.4, the viscosity stabilizer being present during polyamidation in an amount of 0.204-1.63 percent based on the weight of the polyamide.

2. A wet-spun filament having improved tensile properties and abrasion resistance made from an aromatic polyamide of the formula



wherein n is indicative of the molecular weight, viscosity-stabilized with N,N-dimethyl formamide, the inherent viscosity of the polyamide being in the range of 1.8 and 2.2, and the said formamide being present during polyamidation in an amount of 0.53-1.22 percent based on the weight of the polyamide.

3. A wet-spun filament having improved tensile properties and abrasion resistance made from an aromatic polyamide of the formula



wherein n is indicative of the molecular weight, viscosity-stabilized with N,N-dimethylformamide, the inherent viscosity of the polyamide being in the range of 1.8 and 2.2 and the said formamide being present during polyamidation in an amount of 0.53-1.22 percent based on the weight of the polyamide.

\* \* \* \* \*